

J. APOZNANSKI.

PROCESS OF MAKING ELECTRODES FOR SECONDARY BATTERIES.

APPLICATION FILED DEC. 14, 1910.

1,114,667.

Patented Oct. 20, 1914.

Fig:1.



Fig:2.



Fig:3.



Witnesses:  
Joseph L. Bisbano,  
J. F. Hagg.

Inventor  
Joseph A. Apoznanski  
By his Attorney C. P. Goepel.

# UNITED STATES PATENT OFFICE.

JOSEPH APOZNANSKI, OF MOSCOW, RUSSIA, ASSIGNOR TO THE FIRM OF STANISLAW & GEORGIJ GASZYNSKI BROS., APOZNANSKI & CO., OF MOSCOW, RUSSIA.

## PROCESS OF MAKING ELECTRODES FOR SECONDARY BATTERIES.

1,114,667.

Specification of Letters Patent.

Patented Oct. 20, 1914.

Application filed December 14, 1910. Serial No. 597,875.

To all whom it may concern:

Be it known that I, JOSEPH APOZNANSKI, a subject of the Czar of Russia, residing in Moscow, in the Empire of Russia, have invented certain new and useful Improvements in Processes of Making Electrodes for Secondary Batteries, of which the following is a specification.

My invention relates to the manufacture of electrodes for secondary batteries, and a primary object is to provide an exceedingly simple process, by which not only an exceptionally large effective capacity of the electrodes is obtained, but simultaneously, besides a great porosity of the same, and considerable durability, even when they are severely discharged.

My process is carried into practice as follows: My process is carried out by the aid of apparatus which is shown in the accompanying drawings, in which—

Figure 1 is a vertical longitudinal section showing the oven with banks of plates therein, Fig. 2 is a vertical transverse section on line 2—2 of Fig. 1, and Fig. 3 is a detail view of the arrangement of the plates, grids, paste, etc., while being subjected to the heating process.

In these figures, similar characters of reference indicate corresponding parts, and in which the oven 10 is provided with doors 11 and 12 at the front thereof, and a grate 13 at the lower portion thereof, for the support of the fuel. Supported within the oven 10 is a chamber 15 which is provided with several superposed supporting-plates 16, each of which consists of a plurality of spaced bars 16<sup>a</sup>, so as to permit the heat to pass between the same. The chamber 15 is smaller than the oven casing, and is arranged so as to provide vertical channels 20 and 21 at either side of the chamber 15, and a channel 22 above the same for the passage of the heat produced by the burning of the fuel. After the heat has done its work, it passes out of the chimney 23.

In the chamber 15 and on the support 16 are arranged a plurality of banks, indicated by 25, one of which is clearly shown in Fig. 3. These banks are built up by arranging alternately glass plates 30 and electrodes 33, which electrodes are built up by the lead grids 31 and a paste 32. At the ends of the glass plates and electrodes, a

layer of paste is provided so as to cover up any leaks, which layer is indicated by 34, and on the top of the uppermost glass plate, a weight 40 of lead or any other suitable material is arranged so as to hold down 60 the plates in position. When the electrodes are thus arranged in the manner indicated, they are subjected to the heat in the oven, and the process hereinafter described is carried out. The process is carried out by having always the entire banks placed in the oven and not the single plates. It will be noticed that each one of these banks contains six accumulator plates and seven cover plates. As some gases, as for instance, water vapors, may fill the interior of the chamber 15 on the carrying out of the process, it might sometimes be preferable to have an exhaust pipe exhaust these gases. For this reason, the tube 37 is provided, which enables these water vapors to pass into the chimney 23. In Fig. 3, the bank is shown in approximate natural size.

Lead salts, *e. g.* minium alone or minium mixed with litharge, or merely litharge alone 80 with sulfuric acid and distilled water, are mixed to form a thick paste, to which subsequently is added some glycerin. The quantity of sulfuric acid which is employed is of special importance and is so selected, in proportion 85 to the quantity of water, that when diluted sulfuric acid is mixed with minium the color of the latter does not change. When the paste has been mixed with suitably diluted sulfuric acid a small quantity of sulfuric 90 acid is added but only so much that the color of the minium becomes only immaterially darker. Some glycerin may then be added to the paste, whereupon the paste is ready for being filled into the grid-plates. It is 95 to be noted that when the quantity of sulfuric acid is too great when making the paste, the durability of the plates is considerably impaired.

Before the paste is filled into the grid-plates, it is well heated and only after it has attained a suitable temperature, filled hot into the plates. Not only lead-plates but also carbon-plates may be employed as grids. In the present process it is not necessary to 105 press the filled grid-plates as is otherwise frequently thought to be preferable, and consequently the grids can be made particularly light and thin, which materially contributes toward obtaining a battery of light 110

weight. Immediately after the hot paste has been put into the grids, the latter are dried in a special manner, to wit, by placing them between smooth plates which are not attacked by sulfuric acid, such as glass or enameled iron plates, and then drying them in a heated chamber. The object of placing the plates between acid-proof plates, that is to say, glass or enameled iron plates, is to prevent the admission of air. In the one and in the other case, the temperature at which the plates are dried must be below the melting point of the lead-grid and of the lead salts used for forming the paste. When the drying process is thus carried into practice, the plates are dried very rapidly, and electrodes obtained in which the active material is exceedingly hard and simultaneously also exceptionally porous. After being dried, forming can at once take place, to which end sulfuric acid of 16 to 26 degrees Beaumé is preferably employed. This same electrolyte is also used for the secondary batteries, but I do not desire to be bound to the density just stated. Any desired suitable strength of current may be employed during the forming operation, but the stronger the current which is employed, the more rapidly are the plates formed.

When lead-grids are employed for making the electrodes, the capacity of such a secondary battery is at least 40 ampere-hours per kilogram of electrode, but when carbon-grids are employed, this value rises to 50 and more ampere-hours. It is true that such outputs have been known heretofore, nevertheless they could be obtained only by specially complicated means and at the expense of the durability of the battery. In contradistinction thereto, as mentioned above, my process of manufacture is particularly simple, the plates in themselves have the appearance of an ordinary electrode and their durability is exceptionally great. The active material as such possesses, besides great porosity, great hardness and resistance, while the lead or carbon-grids, serving less for strengthening the electrodes, but mainly as the conductors of the current, can therefore be made exceedingly light, so that the entire

secondary battery is materially diminished in weight.

The invention consists therefore of the improved step in the art, as also the improved process embodying said step, which consists in drying the paste filled in the grids and preventing the gases from free exit from the grids during such drying, such drying being carried out very rapidly and at a temperature higher than that of the paste, as has been hereinbefore described, and as will be pointed out in the appended claims.

I claim:

1. That step in the herein described process of making electrodes for secondary batteries, which consists in very rapidly drying the paste filled in the grids, and impeding the exit of the gases within the grids during such drying. 65

2. The process herein described of making electrodes for secondary batteries, which consists in drying the paste filled in the grids, and preventing the gases from free exit from the grids during such drying, such drying being carried out very rapidly and 75 at a temperature higher than that of the paste.

3. The process herein described of making electrodes for secondary batteries, which consists in filling the grids with a pasty mass, and thereafter drying them very rapidly while between plates, whereby the gases formed by the drying are prevented from free exit. 80

4. The process herein described of making electrodes for secondary batteries, which consists in filling the grids with a pasty mass, covering the exposed surfaces of the paste filled in the grids, and drying the paste in the grids while so covered, whereby the 90 gases formed during drying are prevented from free exit at the parts so covered.

In testimony, that I claim the foregoing as my invention, I have signed my name in presence of two subscribing witnesses.

JOSEPH APOZNANSKI.

Witnesses:

STANISLAS GASZYNISKI,  
JEHSCAL BOJAR.